# EUROPEAN PATENT SPECIFICATION

(11) **EP 0 661 159 B1**
(45) Date of publication and mention of the grant of the patent: **18.03.1998**
(21) Application number: 93310609.8
(22) Date of filing: 29.12.1993
(51) Int. Cl.: B41J 2/175, B65D 81/26

(54) **Foam-filled aqueous liquid container**
Mit Schaumstoff gefüllte Behälter für wässrige Flüssigkeiten
Récipient rempli de mousse pour liquide aqueux

(43) Date of publication of application: 05.07.1995
(73) Proprietor: BRIDGESTONE CORPORATION, Tokyo 104 (JP)
(72) Inventor: Yasunaga, Kuniaki, c/o Bridgestone Corp., Yokohama-shi, Kanagawa-ken (JP); Hasegawa, Hajime, c/o Bridgestone Corp., Yokohama-shi, Kanagawa-ken (JP); Kimijima, Isao, Yokohama-shi, Kanagawa-ken (JP)
(74) Representative: Stoner, Gerard Patrick

(56) References cited:
- EP-A- 0 520 695
- US-A- 4 088 132

## Description

This invention relates to a container for aqueous liquid, and more particularly, to a container having a liquid retainer received therein for storing an aqueous liquid, typically an ink retainer for storing an aqueous ink for providing an ink supply to a printing head. The invention also relates to a method of making such a container.

Most liquid containers are stationary, but some are used in a movable state. As a container moves back and forth in a horizontal direction, or up and down in a vertical direction, waves in the liquid give rise to sloshing in the container. If liquid in the container is waving and sloshing it is difficult to discharge liquid from the container at a constant flow rate.

One known solution to this problem is to place a flexible polyurethane foam in a container as a liquid retainer for preventing waving motion of liquid. For example, Japanese Patent Publication No. 2103/1967 discloses such a container. A flexible polyurethane foam is placed in the container for accommodating liquid. Even if the container is used under dynamic conditions, substantial motion of the liquid therein is avoided.

This technique, however, has several drawbacks. In general, flexible polyurethane foams used in such application have about 5 to 20 cells/25 mm. If such a polyurethane foam having a volume corresponding to the interior volume of the container is placed in the container, the foam has relatively weak capillary action and a poor liquid retention capacity. The container thus allows for more or less motion of liquid in dynamic operating conditions so that no consistent delivery of liquid therefrom is expected. This container does not provide a full solution to the above-mentioned problem.

The problem becomes serious particularly with ink retainers used for feeding ink to printing heads. The field of business machine printers now sees a switch from the wire dot and thermal transfer printing systems to the ink jet and laser beam printing systems. In the ink jet printing system, aqueous ink is generally used and an ink retainer is typically inserted in a container in order to retain the ink uniformly in the container. Without such an ink retainer it is difficult to feed ink at a constant rate, because the feed rate can vary with the residual amount of ink in the container. In a printing system wherein the ink container moves with the printing head, the ink constantly waves and sloshes in the container, hindering constant ink supply.

For such ink containers, ink retainers are essential and are generally made of flexible polyurethane foam. Polyurethane foams as produced possess thin cell membranes; those polyurethane foams from which the cell membranes have been removed e.g. by heating are often used. Typically such polyurethane foams are installed in the containers in a compressed state. As a result of compression, the foams have an increased density of cells which is advantageous for ink retention. An example of such a container is described in EP-A-520695.

Regrettably, from the standpoint of a manufacturing process it is rather difficult to compress and insert polyurethane foam into containers. Often the foam is received in a partially turned over or wrinkled state; only a few foams are inserted properly. If the polyurethane foam received in the container is locally deformed, the deformation can form a path for ink. In some cases, such deformation can form a shortcut air flowpath from a vent to an exit port of the container, allowing air to reach the exit port directly and inhibiting further ink supply despite the ink being available in the container.

### SUMMARY OF THE INVENTION

Therefore, an object of the present invention is to provide a novel and improved liquid storing container having a flexible polyurethane foam received therein for not only retaining liquid, but also preventing liquid from sloshing when the container is moved so that liquid can be delivered from the container at a constant flow rate.

According to the present invention, there is provided a container having an inner wall defining an interior volume. A flexible polyurethane foam is received in the container for storing an aqueous liquid. The polyurethane foam swells with the liquid. When swollen, the polyurethane foam makes close contact with the container inner wall.

More particularly, the flexible polyurethane foam to be inserted into the container swells with an aqueous liquid to be charged. When the polyurethane foam is initially inserted into the container, the foam need not closely contact the container inner wall. A gap may be left between the foam and the container inner wall, that is, the foam may have a volume slightly smaller than the container interior volume. This looseness facilitates insertion of the foam into the container. The invention is not limited to such a foam of smaller dimensions and a foam which is compressed upon insertion into a container is also acceptable herein.

When the aqueous liquid is introduced into the container, the foam is impregnated and swollen with the liquid so that the foam expands into close contact with the container inner wall. The swollen foam fully occupies the container inner volume and remains uniform. No gap or empty space is left in the container. The ink-swollen or impregnated foam is effective not only to retain liquid but also to prevent liquid from sloshing when the container is moved. It is then possible to deliver liquid from the container at a constant flow rate. Therefore, the container of the invention is particularly useful as an ink retainer container for providing a constant ink supply to a printing head.

The invention also provides a method of manufacturing a container as described above.

### BRIEF DESCRIPTION OF THE DRAWING

The only figure, FIG. 1 is a partially cut-away perspective view of a container according to one embodiment of the invention.

### DETAILED DESCRIPTION

A liquid storage container of the present invention is illustrated in FIG. 1 as comprising a container casing 10 and a liquid retainer 20 placed therein for absorbing and retaining an aqueous liquid.

The material and shape of the container casing 10 may be selected in accordance with a particular purpose of the container. In one preferred embodiment wherein the container is an ink container from which ink is supplied to the printing head, the container casing is of a box shape having an air vent 30 at the top and an ink exit port 32 at the bottom as shown in FIG. 1 and made of any plastic material such as polypropylene.

The liquid retainer 20 is made of flexible polyurethane foam which is swellable with an aqueous liquid to be contained in the container, for example, aqueous ink. The swellable polyurethane foam may be a hydrophilic polyurethane foam if the liquid with which the container is to be charged is aqueous, typically aqueous ink. Such a hydrophilic polyurethane foam is generally obtained by using a polyol including a higher proportion of ethylene oxide than of propylene oxide as one starting reactant for the manufacture of the polyurethane.

A desired swelling factor is obtained by properly selecting various parameters of the polyurethane foam manufacturing process. At least one polyether polyol in which the average weight ratio of ethylene oxide (EO) to propylene oxide (PO) ranges from 20:80 to 50:50 is used as one starting reactant. To 100 parts by weight of the polyether polyol is added 2 to 5 parts by weight of water as a blowing agent. The resulting polyurethane foam will have a desired swelling factor.

More particularly, the polyol component used is a mixture of a first polyether polyol which is obtained by ring-opening polymerization of propylene oxide with glycerin and a second polyether polyol which is obtained by ring-opening polymerization of ethylene oxide and propylene oxide in a weight ratio of 75:25 with glycerin, the first and second polyether polyols being mixed in a weight ratio of from 74:26 to 33:67.

The isocyanate component is preferably selected from tolylene diisocyanate and xylylene diisocyanate. To 100 parts by weight of the polyol component is added 20 to 60 parts by weight of the isocyanate component. A catalyst and a foam stabilizer are also added. The catalysts used herein include amine catalysts such as triethylenediamine and pentamethyldiethylenetriamine and tin catalysts such as stannous octoate and dibutyltin dilaurate and are used in an amount of 0.01 to 1.0 parts by weight. The foam stabilizers include silicone foam stabilizers such as dimethylpolysiloxane having polyether polyol added thereto and are used in an amount of 0.1 to 2.0 parts by weight. Water is added to this mixture as a foaming agent whereupon polyurethane reaction takes place to produce a flexible polyurethane foam.

If the polyurethane foam takes up a large amount of aqueous liquid within itself, the container is reduced in liquid supply efficiency. In this regard, the polyurethane foam should preferably have a swelling factor of 5 to 60% by volume, more preferably 10 to 40% by volume with the aqueous liquid. With a swelling factor of less than 5% by volume, the polyurethane foam must be shaped to closely conform to the container interior, causing difficulty in inserting the foam into the container. Furthermore after admission of aqueous liquid an empty space can be left unoccupied by the swollen foam. Polyurethane foam with a swelling factor of more than 60% by volume would take up too much aqueous liquid, so that the amount of aqueous liquid that can be taken out of the container is reduced and the container becomes an ineffective liquid supplier.

If the polyurethane foam before insertion has a cell diameter sufficient to retain an aqueous liquid without the need for compression, its swelling factor may be relatively low. If the polyurethane foam has a relatively large cell diameter, the foam is preferably inserted into the container in a compressed state insofar as it is possible to take advantage of the swelling property.

The number of cells in the polyurethane foam may be appropriately selected; it is generally 30 to 200 cells/25 mm. For ink retention purposes, foams having 50 to 200 cells/25 mm, especially 70 to 200 cells/25 mm are preferable because such foams can be used as an ink retainer without compression.

The most preferred form of polyurethane foam is an open-cell reticulated urethane foam having no cell membranes.

Of course, a polyurethane foam which must be compressed before it can be inserted into the container is acceptable in the present invention. Even when the foam is in improper state, for example, deformed or wrinkled at the time of insertion, the foam itself can cure such defects as it swells with aqueous ink, becoming a fully effective ink retainer.

### EXAMPLE

Examples of the present invention are given below by way of illustration and not by way of limitation.

### Example 1 & Comparative Example 1

A flexible polyurethane foam (A) was prepared using a polyether polyol formed from propylene oxide alone and having a molecular weight of 3,000 and another polyether polyol having an ethylene oxide/propylene oxide (EO/PO) weight ratio of 75/25 and a molecular weight of 3,000 and tolylene diisocyanate (TDI). In the resulting polyurethane foam, the weight ratio of total EO/PO was 40/60. The polyurethane foam (A) had 60 cells/25 mm and a swelling factor of 15% by volume with water.

Into a transparent plastic container casing defining an interior of 30 mm × 40 mm × 50 mm was inserted a block of polyurethane foam (A) cut to slightly smaller dimensions of 28 mm × 38 mm × 48 mm. The container was then charged with aqueous ink.

The container was visually observed from the outside, noting no empty space at the container inner wall. Ink was slowly discharged from an exit port at the bottom of the container under a constant negative pressure. A constant flow rate could be maintained. No air shortcut path, connecting a vent at the top and the exit port at the bottom, was created.

Comparative Example 1 used a flexible polyurethane foam (B) which had 60 cells/25 mm and was scarcely swellable with water. This polyurethane foam (B) was inserted into the same container as in Example 1. The polyurethane foam (B) was also shaped to conform to the container interior as in Example 1.

An ink discharge test was carried out, with the result that an air shortcut path connecting the vent and the exit port was created along the container inner wall, disturbing smooth ink delivery.

### Examples 2-3 & Comparative Examples 2-3

Tested in these examples were polyurethane foams having a swelling factor with water of less than 3% by volume (Comparative Example 2), 15% by volume (Example 2), 30% by volume (Example 3), and 70% by volume (Comparative Example 3). Before insertion into the container, all the polyurethane foams had 40 cells/25 mm.

Containers had an interior of 30 mm × 40 mm × 50 mm as in Example 1. A polyurethane foam block having a volume 4 times the container interior volume was compressed and inserted into each container.

The containers were then charged with aqueous ink. The behavior of the polyurethane foam was visually observed. In Comparative Example 2 a deformation of the foam, induced upon insertion, remained after ink admission. This was probably because the foam in Comparative Example 2 was scarcely swellable with the ink. In the remaining Examples, the swollen foams appeared satisfactory.

Next, the ink was discharged by suction from the exit port at the bottom at a constant flow rate of 10 ml/min. The suction test was terminated at the point of time when ink delivery from the exit port ceased, that is, when air first came out. The amount of ink sucked up until then was measured.

The suction amount was 49 g and 45 g in Examples 2 and 3, respectively. In Comparative Example 2, the suction amount was as small as 22 g despite a sufficient amount of ink left in the container because an air path was created between the vent and the exit port. Comparative Example 3 performed better than Comparative Example 2, but a large amount of ink was taken up by the polyurethane foam and the suction amount was 32 g.

These results show that when used as an aqueous ink retainer, the polyurethane foam should have a volumetric swelling factor with water between 5% and 60%.

There has been described a container for storing an aqueous liquid, typically aqueous ink in which a flexible polyurethane foam which is swellable with the aqueous liquid is received. Upon insertion of the foam into the container, the foam need not closely conform to the container inner wall. Once the aqueous liquid is admitted into the container, the polyurethane foam swells therewith to come in close contact with the container inner wall. The swollen foam completely occupies the container interior. In an embodiment wherein a polyurethane foam block having a slightly smaller volume than the container interior volume is inserted into the container, charging of the container with an aqueous liquid causes the polyurethane foam to be swollen therewith so that the foam may come in close contact with the container inner wall without leaving a gap.

In swollen state, the foam is not only effective for retaining the aqueous liquid against wavy motion, but also allows the aqueous liquid to be released therefrom if a suction force is applied. Even when the container is moved or swung, the liquid in the container is prevented from sloshing and can be discharged from the exit port at a constant flow rate.

The container of the invention is thus a useful ink reservoir for storing and supplying an aqueous ink to a printing head. It also finds application as tanks to be attached to vehicles.

Although some preferred embodiments have been described, many modifications and variations may be made thereto in the light of the above teachings. It is therefore to be understood that within the scope of the appended claims, the invention may be practiced otherwise than as specifically described.

## Claims

1. A container (10) having a flexible polyurethane foam (20) received therein for storing an aqueous liquid, characterised in that said polyurethane foam (20) swells with aqueous liquid to make close contact with the inner wall of the container (10).

2. A container (10) according to claim 1 wherein said polyurethane foam (20) includes a hydrophilic group.

3. A container (10) according to claim 1 or 2 wherein said polyurethane foam (20) has a swelling factor of 5 to 60% by volume with the aqueous liquid.

4. A container (10) according to claim 1 or 2 wherein said polyurethane foam (20) has a swelling factor of 10 to 40% by volume with the aqueous liquid.

5. A container (10) according to any one of the preceding claims wherein the polyurethane foam (20) has 70 to 200 cells/25 mm.

6. A container according to any one of the preceding claims in which the polyurethane is one made by reacting polyether polyol with an isocyanate, the polyether polyol having residues of ethylene oxide (EO) and propylene oxide (PO) with the average weight ratio EO:PO in the range 20:80 to 50:50.

7. A container (10) according to any one of the preceding claims wherein the container is an ink reservoir and the liquid is an aqueous ink.

8. A container (10) according to any one of the preceding claims, wherein in the absence of aqueous liquid said polyurethane foam (20) has a volume smaller than the container (10) inner volume.

9. A method of manufacturing a container according to any one of the preceding claims comprising inserting a polyurethane foam block into the container, and charging the container with an aqueous liquid to cause the foam to swell and make close contact with the inner wall of the container.

10. A method according to claim 8 wherein the polyurethane foam block, on insertion into the container, has a volume smaller than the internal volume of the container and is in a non-compressed state.

## Patentansprüche

1. Behälter (10) mit darin aufgenommenen flexiblem Polyurethanschaum (20) zum Speichern einer wäßrigen Flüssigkeit, dadurch gekennzeichnet, daß der Polyurethanschaum (20) mit wäßriger Flüssigkeit aufquillt, so daß er die Innenwand des Behälters (10) eng berührt.

2. Behälter (10) nach Anspruch 1, worin der Polyurethanschaum (20) eine hydrophile Gruppe enthält.

3. Behälter (10) nach Anspruch 1 oder 2, worin der Polyurethanschaum (20) mit der wäßrigen Flüssigkeit einen Aufquellfaktor von 5 bis 60 Vol.-% aufweist.

4. Behälter (10) nach Anspruch 1 oder 2, worin der Polyurethanschaum (20) mit der wäßrigen Flüssigkeit einen Aufquellfaktor von 10 bis 40 Vol.-% aufweist.

5. Behälter (10) nach einem der vorangegangenen Ansprüche, worin der Polyurethanschaum (20) 70 bis 200 Zellen/25 mm aufweist.

6. Behälter nach einem der vorangegangenen Ansprüche, bei dem das Polyurethan ein durch Umsetzen von Polyetherpolyol mit einem Isocyanat hergestelltes ist, wobei das Polyetherpolyol Ethylenoxid(EO)-reste und Propylenoxid(PO)-reste mit einem durchschnittlichen Gewichtsverhältnis EO:PO im Bereich von 20:80 bis 50:50 aufweist.

7. Behälter (10) nach einem der vorangegangenen Ansprüche, worin der Behälter ein Tintenbehälter und die Flüssigkeit eine wäßrige Tinte ist.

8. Behälter (10) nach einem der vorangegangenen Ansprüche, worin der Polyurethanschaum (20) in Abwesenheit wäßriger Flüssigkeit ein Volumen aufweist, das kleiner als das Innenvolumen des Behälters (10) ist.

9. Verfahren zur Herstellung eines Behälters nach einem der vorangegangenen Ansprüche, umfassend das Einsetzen eines Polyurethanschaumblocks in den Behälter und das Befüllen des Behälters mit einer wäßrigen Flüssigkeit, wodurch bewirkt wird, daß der Schaum aufquillt und in engen Kontakt mit der Innenwand des Behälters kommt.

10. Verfahren nach Anspruch 8, worin der Polyurethanschaumblock beim Einsetzen in den Behälter ein Volumen aufweist, das kleiner als das Innenvolumen des Behälters ist, und sich in einem nichtzusammengedrückten Zustand befindet.

## Revendications

1. Récipient (10) ayant une mousse de polyuréthanne flexible (20) qui y est reçue pour stocker un liquide aqueux, caractérisé en ce que ladite mousse de polyuréthanne (20) gonfle avec le liquide aqueux pour venir en proche contact avec la paroi interne du récipient.(10).

2. Récipient (10) selon la revendication 1, où ladite mousse de polyuréthanne (20) comprend un groupe hydrophile.

3. Récipient (10) selon la revendication 1 ou 2, où ladite mousse de polyuréthanne (20) a un facteur de gonflement de 5 à 60 % en volume avec le liquide aqueux.

4. Récipient (10) selon la revendication 1 ou 2, où ladite mousse de polyuréthanne (20) a un facteur de gonflement de 10 à 40 % en volume avec le liquide aqueux.

5. Récipient (10) selon l'une quelconque des revendications précédentes, où la mousse de polyuréthanne (20) a 70 à 200 alvéoles/25 mm.

6. Récipient selon l'une quelconque des revendications précédentes, dans lequel le polyuréthanne est fait par réaction de polyéther polyol avec un isocyanate, le polyéther polyol ayant des résidus d'oxyde d'éthylène (OE) et d'oxyde de propylène (OP) avec le rapport pondéral moyen de OE:OP compris entre 20:80 et 50:50.

7. Récipient (10) selon l'une quelconque des revendications précédentes où le récipient est un réservoir d'encre et le liquide est une encre aqueuse.

8. Récipient (10) selon l'une quelconque des revendications précédentes où, en l'absence du liquide aqueux, ladite mousse de polyuréthanne (20) a un volume plus petit que le volume interne du récipient (10).

9. Méthode de fabrication d'un récipient selon l'une quelconque des revendications précédentes, consistant à insérer un bloc de mousse de polyuréthanne dans le récipient et à charger le récipient d'un liquide aqueux pour forcer la mousse à gonfler et à venir en proche contact avec la paroi interne du récipient.

10. Méthode selon la revendication 8 où le bloc de mousse de polyuréthanne, à l'insertion dans le récipient, a un volume plus petit que le volume interne du récipient et est à un état non comprimé.
